

# United States Patent Office

3,036,902

Patented May 29, 1962

1

3,036,902

**3,050,502**  
**MOTOR FUEL COMPOSITION**

MOTOR FUEL COMPOSITION  
Martin Hamer, Chicago, Ill., and Sherman R. Oblad,  
Munster, Ind., assignors to Standard Oil Company,  
Chicago, Ill., a corporation of Indiana  
No Drawing. Filed Mar. 3, 1958, Ser. No. 718,490  
6 Claims. (Cl. 44-56)

6 Claims. (Cl. 44—56)

This invention relates to motor fuel compositions and particularly to motor fuel compositions for spark-ignition internal combustion engines adapted to prevent engine stalling due to carburetor icing.

Engine stalling due to carburetor icing occurs most frequently under engine idling conditions and particularly under weather conditions of relatively high humidity and at a temperature below about 60° F. While this problem has been in existence for many years, it has of late become of increased importance because of recent engine design. Most post-war cars are provided with automatic chokes and provide no means for manual operation of the throttle so that operators of such cars are no longer able to regulate idle speeds during warm-up periods to prevent stalling. Furthermore, the idle speed of automobiles equipped with automatic transmissions is rather critical during the warm-up period and the fastest idle rate which may be used is limited to avoid creeping. Another factor in carburetor icing is the high volatility of motor fuels now provided for present-day engines.

It has been established that the cause of engine stalling in cool humid weather is the formation of ice in the engine carburetor. On such cool moist days, the gasoline evaporated in the carburetor produces a sufficient refrigerating effect to condense and freeze the moisture present in the air entering the carburetor. Fuel vaporization in the fuel carburetor under such conditions can cause a temperature drop in the carburetor of up to 50° F. below that of the entering air; as a result, up to the time of complete engine and radiator warm-up, this drop in temperature causes formation of ice crystals in the carburetor. The maximum refrigeration of the type referred to takes place under conditions of light load operation. As cooling of the carburetor parts takes place, ice begins to form as soon as these parts are refrigerated to a temperature below about 30° F., so that, when the throttle is closed to the idle position, the ice forms, formed or forming in the carburetor, particularly that formed, on the throttle plate and the adjacent walls, closes the narrow air ports, thereby restricting the normal flow of the air to the engine, causing repeated engine stalling. While an engine stalled, because of carburetor icing, can be readily started because the ice formed melts almost immediately due to residual heat from the exhaust manifold, it is highly desired to avoid any stalling due to carburetor icing because of the attendant inconvenience. For example, stalling due to carburetor icing of a car, equipped with automatic transmission, frequently does not occur until the driver is ready to accelerate so that at this most inconvenient time it is necessary to shift the car to neutral, restart the engine and shift back into gear, all of which magnifies the inconvenience of frequent stalls.

It is an object of the present invention to provide a motor fuel for a spark-ignition internal combustion engine which will prevent carburetor icing. Another object of the invention is to provide gasoline for spark-ignition internal combustion engines which will prevent the accumulation of ice crystals on carburetor parts during idling speed and under conditions of light load operation. Still another object of the invention is to provide a hydrocarbon motor fuel composition for spark-ignition internal combustion engines which will prevent engine stalling.

2

due to carburetor icing. Other objects and advantages of the present invention will become apparent from the following description thereof.

In accordance with the present invention, the foregoing objects can be attained by incorporating in the motor fuel for spark-ignition combustion engines from about 0.005% to about 0.5% of a substituted imidazoline, more fully defined hereinafter, and in combination therewith from about 0.01% to about 3.0% of an alkanol having from 1 to about 4 carbon atoms, such as methanol, ethanol, isopropanol, propanol, 1-butanol, 2-butanol, 2-methyl-2-propanol and isobutanol. If desired, mixtures of such alkanols can be used.

The substituted imidzoline used in this invention can be represented by the following probable general structure:



25 in which R is an alkyl, alkenyl or alkadienyl group or mixtures thereof, having from about 10 to about 24 carbon atoms, and X is a polar group such as hydroxy, amino, carboxyl or an alkyl group containing one of such polar group.

The imidazolines (or glyoxalidine) employed are made by well known methods such as described in Wilson U.S. No. 2,267,965 and Wilkes U.S. No. 2,214,152. Briefly, the method involves reacting a fatty acid with an aliphatic polyamine with the elimination of water.

Specific examples of imidazolines suitable for use in the present invention include 1-hydroxyethyl-2-heptadecenyl imidazoline, 1-aminoethyl-2-undecyl imidazoline, 1-hydroxyethyl-2-pentadecyl imidazoline, 1-aminoethyl-2-heptadecenyl imidazoline, 1-aminoethyl-2-heptadecyl imidazoline, 1-hydroxyethyl-2-heptadecyl imidazoline, 1-(aminoethyl ethylamino)-2-heptadecenyl imidazoline, and the like.

Several commercial imidazoline compounds are available which can be used in the preparation of the above salts. Examples of such commercial products are "Amine O," "Amine 220," and "Nalcamine G-12," all of which contain R groups (above structure) of 17 carbon atoms and a hydroxyl polar group (X in the above structure). Another commercial imidazoline is "Nalcamine G-39M" which has the same R group but contains  $-\text{NH}_2$  in its polar side group (X).

50 The de-icer combination of the present invention can be used in any hydrocarbon motor fuel in the gasoline boiling range adapted for use in spark-ignition internal combustion engines. Such hydrocarbon motor fuels adapted to be used in the fall or spring (intermediate) 55 and in the winter months when stalling due to carburetor icing is most prevalent, have an ASTM initial boiling point of about 90-80° F., a 90% off distillation temperature of not more than about 365-356° F. respectively and an end point of not more than about 415° F. 60 Typical gasoline inspections are illustrated by the following:

|                              | Intermediate | Winter |
|------------------------------|--------------|--------|
| 65 Initial Boiling Point ° F | 88           | 80     |
| 10% Recovery, ° F            | 123          | 108    |
| 50% Recovery, ° F            | 210          | 197    |
| 90% Recovery, ° F            | 312          | 309    |
| End Point ° F                | 373          | 364    |

70 The hydrocarbon motor fuel can contain any of the commonly used additives such as lead alkyl anti-knock agents, e.g. tetraethyl lead, lead scavenging agents, dyes,



UNITED STATES PATENT OFFICE  
CERTIFICATE OF CORRECTION

Patent No. 3,036,902

May 29, 1962

Martin Hamer et al.

It is hereby certified that error appears in the above numbered patent requiring correction and that the said Letters Patent should read as corrected below.

Column 2, line 7, for "0.5%" read -- 0.05% --; line 14, for "imidzoline" read -- imidazoline --; column 4, line 35, for "to", second occurrence, read -- of --.

Signed and sealed this 4th day of September 1962.

(SEAL)

Attest:

ERNEST W. SWIDER

Attesting Officer

DAVID L. LADD

Commissioner of Patents